# EUROPEAN PATENT SPECIFICATION

(11) **EP 2 083 928 B1**
(45) Date of publication and mention of the grant of the patent: **26.10.2011**
(21) Application number: 07864530.6
(22) Date of filing: 16.11.2007
(51) Int. Cl.: A63B 51/02, D02G 3/44, G10D 3/10, D07B 1/02

(54) **Buffer layer for strings**
Pufferschicht für Saiten
Couche tampon pour cordons

(30) Priority: 16.11.2006 US 866199 P
(43) Date of publication of application: 05.08.2009
(73) Proprietor: Applied Nanotech Holdings, Inc., Austin, TX 78758-7631 (US)
(72) Inventor: YANIV, Zvi, Austin, TX 78746 (US); LI, Yunjun, Austin, Texas 78759 (US); MAO, Dongsheng, Austin, Texas 78732 (US)
(74) Representative: Harrison Goddard Foote
(86) International application number: PCT/US2007/084973
(87) International publication number: WO 2008/061229

(56) References cited:
- EP-A- 1 574 234
- US-A1- 2003 143 396
- US-A1- 2003 145 574
- US-A1- 2004 096 389
- US-B1- 6 460 321

## Description

### BACKGROUND

The strings for sports equipment (e.g., tennis racquets) or musical instruments are usually coated with a thin layer at their outmost surface to improve their durability, spin, feeling, etc. Polyamide (nylon), polyester, and other polymers have been used to coat on strings. Nanocomposites, such as clay and carbon nanotube reinforced nylon 6 nanocomposites, having better physical properties than neat nylon 6, are of a potential to be highly durable string coating materials with other functionalities. The reinforcing polymeric composites using nano-sized clay particles with high aspect ratio have been investigated since the 1980's (see U.S. Patent No. 4,739,007). Strings are usually polymer materials with a multi-layer structure - core filament, wrapping filaments on the core filament, and coating. For the strings with multi-layer structures, coating materials are required to match the base materials and have good melt-flow properties (acceptable viscosity) at certain temperature to allow them to be penetrated into the gaps between the wrapping filaments. Viscosity of a nanocomposite is usually higher than neat nylon 6 at the same temperature. Thus, the nanocomposite may not easily penetrate into the gaps between the wrapping filaments. Figure 1 shows an SEM image of a cross-section view of a nylon 6/clay nanocomposite coated on a wrapping filament. It can be seen that the nanocomposite material did not successfully fill out the gaps. Many defects were left in the string which will result in unacceptable durability of the strings. The gaps will result in chipping-off or unacceptable durability of coatings during high impact hitting of balls. More over, due to creation of the gaps, coatings also fail to a fix the filaments on the core materials of the string. Figure 2 shows the chipped materials from filaments and coatings after high impact tests on the strings.

US 6,460,321 discloses a racquet string comprising a core surrounded by at least one sheath, having a plurality of sheath fibres wound around said core, and a coating resin uniting the core and sheath fibres into a unitary body. The sheath fibres are helically wound about the core at a high wind angle, i.e., at a wind angle between 25 and 40 degrees relative to the core axis. Preferably, the sheath comprises a plurality of main sheath fibres and a plurality of non-main sheath fibres, and the core, the main sheath fibres, and the coating resin are transparent. Preferably, the non-main sheath fibres have a relatively low transparency. In this manner, the non-main fibres produce a multi-helix appearance when the string is observed from the side.

### SUMMARY OF THE INVENTION

The present invention provides a string for sports equipment (e.g. tennis rackets) or musical instruments, comprising a core filament wrapped with a plurality of wrapping filaments of a smaller diameter than the core filament, characterized by the following combination: a buffer layer coating filling in gaps between the wrapping filaments and between the wrapping filaments and the core filament, the buffer layer coating being a melt extruded nylon; and an outer composite coating covering over the buffer layer coating, wrapping filaments and core filament, wherein the outer composite coating comprises a composite of nylon and a material selected from clay, carbon nanotubes, ceramic particles such as SiO₂ and Al₂O₃, or glass particles

### BRIEF DESCRIPTION OF THE DRAWINGS

Figure 1 shows an SEM image of a cross-section view of a nylon 6/clay nanocomposite coated on a wrapping filament;
Figure 2 shows an SEM image of chipped materials from filaments and coatings after high impact tests on a string;
Figure 3A illustrates a cross-section of a core filament with wrapping filaments surrounding it;
Figure 3B illustrates a buffer layer applied onto the wrapping filament;
Figure 3C illustrates a coating applied onto the buffer layer; and
Figure 4 illustrates another embodiment of the present invention.

### DETAILED DESCRIPTION

Although polymer nanocomposites have higher physical/mechanical properties than neat polymer materials, they normally have higher viscosity or melt-flow during an extrusion or coating process. To solve this problem, a thin buffer layer is used to coat on the multi-filament wrapped string to fill the gaps. The polymers of the buffer-layer coating have a high melt-flow (low viscosity) during coating process to fill all the gaps between the filaments, and the filaments are fixed by the coatings onto base core materials. More particularly, the invention provides a string for sports equipment (e.g. tennis rackets) or musical instruments as described above under the heading "Summary of the Invention".

### Example 1: A coating system with a nylon 6 buffer layer

Figure 3A illustrates a cross-section of a string for coating comprised of one monofilament core 301 wrapped with smaller-diameter multi-filaments 302. Neat nylon 6 pellets as may be obtained from UBE Industries Inc. (product name: UBE SF 1018 A) are melted. The buffer layer coating 303 is applied by an extrusion process at temperatures ranging from 220°C to 270°C. The thickness of the buffer layer 303 may be from 10 to 100 micrometers. The gaps between the multi-filaments 302 are fully filled by the neat nylon 6 coating.

A wear-resistant coating 304 is then coated (Figure 3C) by an extrusion process at temperatures ranging from 240°C to 280°C. A nylon 6/clay or nylon 6/carbon nanotube nanocomposite may be employed as the wear-resistant coating material 304. The nylon 6 nanocomposite produced by in-situ polymerization may contain 4% nano-clay filler. Other nylon 6 nanocomposites produced by melt-compounded process may also be used for the wear-resistant coatings 304. Except for the clay, carbon nanotubes, ceramic particles such as SiO₂ and Al₂O₃, or glass particles may be used to make nylon6 nanocomposites. The Nylon 6 nanocomposites may also be modified by rubber modifiers to improve the ductility and toughness. The thickness of the wear-resistant coating may be from 1 to 100 micrometers.

### Example 2: A coating system with a nylon 11 buffer layer

Again referring to Figure 3A, the string for coating is one monofilament core 301 wrapped with smaller-diameter multi-filaments 302. Neat nylon 11 may be obtained from ARKEMA Inc. Nylon 11 has a very good melt flow at temperatures over 220°C. Good impact strength and shear strength also make nylon 11 a good buffer layer material. In Figure 3B, the buffer layer coating 303 is applied by an extrusion process at temperatures ranging from 190°C to 270°C.

The thickness of the buffer layer 303 may be from 10 to 100 micrometers. The gaps between the multi-filaments 302 are fully filled by the neat nylon 11 coating.

Referring to Figure 3C, a wear-resistant coating 304 is then coated by an extrusion process at temperatures ranging from 240°C to 280°C. Nylon 6/clay or a nylon 6/carbon nanotube nanocomposite may be employed as the wear-resistant coating material 304. The nylon 6 nanocomposite produced by in-situ polymerization may contain 4% nano-clay filler. Other nylon 6 nanocomposites produced by melt-compounded process may also be used for the wear-resistant coating 304. The nylon 6 nanocomposites may also be modified by rubber modifiers to improve the ductility and toughness. The thickness of the wear-resistant coating 304 may be from 1 to 100 micrometers.

Except for the extrusion process to deposit a coating on the string, other methods such as spraying, dipping, spin coating, brushing, painting, and immersing processes can be used to deposit a coating on the surface of strings. Nylon 6 nanocomposites may be melted at higher than 190°C and extruded to deposit a coating on the strings. Nylon 6 nanocomposites may be dissolved in a solvent such as formic acid and sprayed, dipped, spin coated, brushed, painted, or immersed to deposit a coating on the string at room temperature or elevated temperatures. The solvent may be then removed by a follow-up process such as an evaporation method.

Figure 4 illustrates another embodiment of the present invention. Essentially, the coated string structure of Figure 3C is then coated again with smaller-diameter multi-filaments 401. A buffer layer coating 402, similar to layer 303, is applied by an extrusion process at temperatures ranging from 190°C to 270°C. The thickness of the buffer layer 402 may be from 10 to 100 micrometers. The gaps between the multi-filaments 401 are fully filled by the neat nylon 11 1 coating. A wear-resistant coating 403 is then coated by an extrusion process at temperatures ranging from 240°C to 280°C. Nylon 6/clay or a nylon 6/carbon nanotube nanocomposite may be employed as the wear-resistant coating material 403. The nylon 6 nanocomposite produced by in-situ polymerization may contain 4% nano-clay filler. Other nylon 6 nanocomposites produced by melt-compounded process may also be used for the wear-resistant coating 403. The nylon 6 nanocomposites may also be modified by rubber modifiers to improve the ductility and toughness. The thickness of the wear-resistant coating 403 may be from 1 to 100 micrometers.

## Claims

1. A string for sports equipment (e.g. tennis rackets) or musical instruments, comprising a core filament (301) wrapped with a plurality of wrapping filaments (302) of a smaller diameter than the core filament, **characterized by** the following combination:
a buffer layer coating (303) filling in gaps between the wrapping filaments (302) and between the wrapping filaments (302) and the core filament (301), the buffer layer coating (303) being a melt extruded nylon; and
an outer composite coating (304) covering over the buffer layer coating (303), wrapping filaments (302) and core filament (301), wherein the outer composite coating (304) comprises a composite of nylon and a material selected from clay, carbon nanotubes, ceramic particles such as SiO₂ and Al₂O₃, or glass particles.

2. The string of claim 1, wherein the buffer layer coating (303) comprises nylon 6 or nylon 11.

3. The string of claim 1 or claim 2, wherein the outer coating (304) comprises a composite of nylon and clay nanoparticles or a composite of nylon and carbon nanotubes.

4. The string of claim 3, wherein the outer coating (303) further comprises a rubber modifier.

5. The string of claim 1, further comprising:
another plurality of wrapping filaments (401) wrapped around the outer coating;
another buffer layer coating (402) filling in gaps between the another plurality of wrapping filaments; and
another outer coating covering (403) over the another buffer layer coating.

6. The string of any preceding claim, wherein the nylon buffer layer is between 10 and 100 micrometers thick.

7. The string of any preceding claim, wherein the coating (304) is between 1 and 100 micrometers thick.

8. The string of claim 1, wherein the outer coating (304) comprises a composite of nylon and glass particles or a composite of nylon and ceramic particles.

9. A method for coating a string for sports equipment (e.g. tennis rackets) or musical instruments, comprising wrapping a core filament (301) having a first diameter with one or more wrapping filaments (302) having a second diameter that is less than the first diameter; **characterized in that** the method further comprises:
extruding a melted nylon (303) into gaps between the one or more wrapping filaments (302) and into gaps between the wrapping filaments (302) and the core filament (301); and
extruding a composite coating (304) on a circumference of the string so that it covers the one or more wrapping filaments (302) and the melted nylon (303) in the gaps, wherein the composite coating (304) comprises a composite of nylon and clay nanoparticles, or a composite of nylon and carbon nanotubes, or a composite of nylon and ceramic particles, or a composite of nylon and glass particles.

10. The method of claim 9, wherein the melted nylon (303) comprises nylon 6 or nylon 11.

11. The method of claim 9 or claim 10, wherein the outer coating (304) comprises a composite of nylon and clay nanoparticles or a composite of nylon and carbon nanotubes.

12. The method of claim 11, wherein the outer coating (303) further comprises a rubber modifier.

13. The method of any of claims 9 to 12, wherein the nylon buffer layer is between 10 and 100 micrometers thick.

14. The method of any of claims 9 to 13, wherein the coating (304) is between 1 and 100 micrometers thick.

15. The method of claim 9, wherein the outer coating (304) comprises a composite of nylon and glass particles or a composite of nylon and ceramic particles.

## Patentansprüche

1. Saite für Sportgeräte (z.B. Tennisschläger) oder Musikinstrumente, wobei die Saite eine Seele (301) umfasst, die mit einer Mehrzahl von Mantelfasern (302) mit geringerem Durchmesser als die Seele umwickelt ist, **gekennzeichnet durch** die folgende Kombination:
einen Pufferschichtüberzug (303), der Zwischenräume zwischen den Mantelfasern (302) und zwischen den Mantelfasern (302) und der Seele (301) füllt, wobei es sich bei dem Pufferschichtüberzug (303) um schmelzgesponnenes Nylon handelt; und
einen äußeren Verbundstoffüberzug (304), der den Pufferschichtüberzug (303), die Mantelfasern (302) und die Seele (301) bedeckt, wobei der äußere Verbundstoffüberzug (304) einen Verbundstoff aus Nylon und einem Material umfasst, das aus Ton, Kohlenstoffnanoröhren, Keramikteilchen wie SiO₂ und Al₂O₃ oder Glasteilchen ausgewählt wird.

2. Saite nach Anspruch 1, wobei der Pufferschichtüberzug (303) Nylon 6 oder Nylon 11 1 umfasst.

3. Saite nach Anspruch 1 oder Anspruch 2, wobei der äußere Überzug (304) einen Verbundstoff aus Nylon und Ton-Nanopartikeln oder einen Verbundstoff aus Nylon und Kohlenstoffnanoröhren umfasst.

4. Saite nach Anspruch 3, wobei der äußere Überzug (303) ferner einen Gummimodifikator umfasst.

5. Saite nach Anspruch 1, wobei diese ferner folgendes umfasst:
eine weitere Mehrzahl von Mantelfasern (401), die um den äußeren Überzug gewickelt sind;
einen weiteren Pufferschichtüberzug (402), der Zwischenräume zwischen der weiteren Mehrzahl von Mantelfasern füllt; und
einen weiteren äußeren Überzug (403), der den weiteren Pufferschichtüberzug bedeckt.

6. Saite nach einem der vorstehenden Ansprüche, wobei die Nylonpufferschicht eine Dicke zwischen 10 und 100 Mikrometern aufweist.

7. Saite nach einem der vorstehenden Ansprüche, wobei der Überzug (304) eine Dicke zwischen 1 und 100 Mikrometern aufweist.

8. Saite nach Anspruch 1, wobei der äußere Überzug (304) einen Verbundstoff aus Nylon und Glasteilchen oder einen Verbundstoff aus Nylon und Keramikteilchen umfasst.

9. Verfahren zur Beschichtung einer Saite für Sportgeräte (z.B. Tennisschläger) oder Musikinstrumente, wobei das Verfahren das Umwickeln einer Seele (301) mit einem ersten Durchmesser mit einer oder mehreren Mantelfasern (302) mit einem zweiten Durchmesser umfasst, der kleiner ist als der erste Durchmesser, **dadurch gekennzeichnet, dass** das Verfahren ferner folgendes umfasst:
das Extrudieren von geschmolzenem Nylon (303) in Zwischenräume zwischen der einen oder den mehreren Mantelfasern (302) und in Zwischenräume zwischen den Mantelfasern (302) und Seele (301); und
das Extrudieren eines äußeren Verbundstoffüberzugs (304) an einem Umfang der Saite, so dass dieser die eine oder mehreren Mantelfasern (302) und das geschmolzene Nylon (303) in den Zwischenräumen bedeckt, wobei der Verbundstoffüberzug (304) einen Verbundstoff aus Nylon und Ton-Nanopartikeln oder einen Verbundstoff aus Nylon und Kohlenstoffnanoröhren, oder einen Verbundstoff aus Nylon und Keramikteilchen, oder einen Verbundstoff aus Nylon und Glasteilchen umfasst.

10. Verfahren nach Anspruch 9, wobei das geschmolzene Nylon (303) Nylon 6 oder Nylon 11 umfasst.

11. Verfahren nach Anspruch 9 oder Anspruch 10, wobei der äußere Überzug (304) einen Verbundstoff aus Nylon und Ton-Nanopartikeln oder einen Verbundstoff aus Nylon und Kohlenstoffnanoröhren umfasst.

12. Verfahren nach Anspruch 11, wobei der äußere Überzug (303) einen Gummimodifikator umfasst.

13. Verfahren nach einem der Ansprüche 9 bis 12, wobei Nylonpufferschicht eine Dicke zwischen 10 und 100 Mikrometern aufweist.

14. Verfahren nach einem der Ansprüche 9 bis 13, wobei der Überzug (304) eine Dicke zwischen 1 und 100 Mikrometern aufweist.

15. Verfahren nach Anspruch 9, wobei der äußere Überzug (304) einen Verbundstoff aus Nylon und Glasteilchen oder einen Verbundstoff aus Nylon und Keramikteilchen umfasst.

## Revendications

1. Corde pour équipements sportifs (par exemple, raquettes de tennis) ou instruments de musique, comprenant un filament guipé (301) qui est guipé avec une pluralité de filaments de guipage (302) d'un diamètre plus petit que le filament guipé, **caractérisé par** la combinaison suivante :
un revêtement de couche tampon (303) comblant les espaces entre les filaments de guipage (302) et entre les filaments de guipage (302) et le filament guipé (301), le revêtement de couche tampon (303) étant un nylon extrudé fondu ; et
un revêtement composite externe (304) recouvrant le revêtement de couche tampon (303), les filaments de guipage (302) et le filament guipé (301), dans laquelle le revêtement composite externe (304) comprend un composite de nylon et d'un matériau choisi dans le groupe constitué d'argile, de nanotubes de carbone, de particules de céramique telles que SiO₂ et Al₂O₃, ou de particules de verre.

2. Corde selon la revendication 1, dans laquelle le revêtement de couche tampon (303) comprend du nylon 6 ou du nylon 11.

3. Corde selon la revendication 1 ou 2, dans laquelle le revêtement externe (304) comprend un composite de nylon et de nanoparticules d'argile ou un composite de nylon et de nanotubes de carbone.

4. Corde selon la revendication 3, dans laquelle le revêtement externe (303) comprend en outre un modificateur de caoutchouc.

5. Corde selon la revendication 1, comprenant en outre :
une autre pluralité de filaments de guipage (401) guipés autour du revêtement externe ;
un autre revêtement de couche tampon (402) comblant les espaces entre l'autre pluralité de filaments de guipage ; et
un autre revêtement externe (403) couvrant l'autre revêtement de couche tampon.

6. Corde selon l'une quelconque des revendications précédentes, dans laquelle la couche tampon en nylon est comprise entre 10 et 100 micromètres d'épaisseur.

7. Corde selon l'une quelconque des revendications précédentes, dans laquelle le revêtement (304) est compris entre 1 et 100 micromètres d'épaisseur.

8. Corde selon la revendication 1, dans laquelle le revêtement externe (304) comprend un composite de nylon et de particules de verre ou un composite de nylon et de particules de céramique.

9. Procédé de revêtement d'une corde pour équipements sportifs (par exemple, raquettes de tennis) ou instruments de musique, comprenant l'étape consistant à guiper un filament guipé (301) ayant un premier diamètre avec un ou plusieurs filaments de guipage (302) ayant un second diamètre qui est inférieur au premier diamètre ; **caractérisé en ce que** le procédé comprend en outre les étapes consistant à :
extruder un nylon fondu (303) dans les espaces entre le ou les filaments de guipage (302) et dans les espaces entre les filaments de guipage (302) et le filament guipé (301) ; et
extruder un revêtement composite (304) sur une circonférence de la corde de sorte qu'il couvre le ou les filaments de guipage (302) et le nylon fondu (303) dans les espaces, dans laquelle le revêtement composite (304) comprend un composite de nylon et de nanoparticules d'argile, un composite de nylon ou de nanotubes de carbone, un composite de nylon et de particules de céramique, ou un composite de nylon et de particules de verre.

10. Procédé selon la revendication 9, dans lequel le nylon fondu (303) comprend du nylon 6 ou du nylon 11.

11. Procédé selon la revendication 9 ou 10, dans lequel le revêtement externe (304) comprend un composite de nylon et de nanoparticules d'argile ou un composite de nylon et de nanotubes de carbone.

12. Procédé selon la revendication 11, dans lequel le revêtement externe (303) comprend en outre un modificateur de caoutchouc.

13. Procédé selon l'une quelconque des revendications 9 à 12, dans lequel la couche tampon en nylon est comprise entre 10 et 100 micromètres d'épaisseur.

14. Procédé selon l'une quelconque des revendications 9 à 13, dans lequel le revêtement (304) est compris entre 1 et 100 micromètres d'épaisseur.

15. Procédé selon la revendication 9, dans lequel le revêtement externe (304) comprend un composite de nylon et de particules de verre ou un composite de nylon et de particules de céramique.
